

## UNITED STATES PATENT OFFICE

JOHN W. WALTON, OF ROCKDALE, TENNESSEE, ASSIGNOR TO TENNESSEE PRODUCTS CORPORATION, OF NASHVILLE, TENNESSEE, A CORPORATION OF TENNESSEE

## PROCESS OF PRODUCING PHOSPHORUS

No Drawing.

Application filed September 22, 1927. Serial No. 221,401.

This invention relates to improvements in processes for producing phosphorus and more particularly to a method of recovering phosphorus from a blast furnace as a by-product in the production of ferro-phosphorus.

As well known to those skilled in the art, ferro-phosphorus is an alloy of iron and phosphorus and is ordinarily produced by the treatment of phosphate rock, coke and iron bearing materials in a blast furnace. As is common in blast furnace operations, the raw materials are charged into the furnace and the ferro-phosphorus withdrawn periodical-  
ly in a molten state along with slag, the gases passing out through a down-comer near the top of the furnace stack and utilized in generation of power. These gases are known to contain phosphorus, which is capable of recovery, would prove to be a valuable by-product in the production of ferro-phosphorus. Attempts have been made to remove the phosphorus from the furnace gases near the top of the furnace, but these attempts have not been successful from a commercial standpoint owing to operating difficulties encountered, such as the clogging or bridging over of the material at the top of the stack. Moreover, the gases near the top of the furnace are laden with impurities aside from containing relatively small quantities of phosphorus, with the result that if recovered in any appreciable amounts, it is generally accompanied by considerable quantities of these impurities which can only be removed at great expense and extensive equipment for the purpose.

The object of the present invention is, therefore, to provide an economical and com-  
merically practical method of recovering the phosphorus in relatively large quantities and in a relatively pure state from a blast furnace, and more especially as a by-product of ferro-phosphorus production operations. The manner in which the operations are carried out will be understood from the following:

Experience in ferro-phosphorus blast furnace operations has led to the conclusion that there exists two fairly well defined melting zones in the furnace,—one in which the iron

ore is smelted and another in which the phosphate rock melts or is fused. It has also been established that the phosphate rock requires a higher temperature for reduction than does the iron ore, and hence the melting zone of 55 the phosphate rock is below that of the iron ore, and in the region adjacent the tuyères where the maximum temperature is maintained. As well known in the blast furnace art, the tuyères are the openings through 60 which an air blast is admitted to the furnace, and are located in the lower portion of the stack but above the bottom thereof. Thus as the charge of raw materials ordinarily consisting of phosphate rock, iron-ore, coke and 65 a flux, descends in the stack, the reduction of the iron oxide in the charge takes place at a higher level, but the phosphate rock is not reduced until it reaches a lower level of highest temperature where it comes into contact 70 with the incandescent coke, thus liberating the phosphorus which is carried upwardly by the gases containing carbon monoxide and phosphorus. The ascending gases encounter the iron in the process of reduction in the upper parts of the stack whereupon the major portion of the phosphorus is absorbed and the remainder with the carbon monoxide passing on and upwardly to the top of the stack and thence to the down-comer. Hence 75 as the gases reach a higher level, they become leaner in phosphorus content, until eventually they escape with little or no phosphorus. On the other hand, the gases at the lower level of the stack are rich in phosphorus and manifestly so, since the gases have not had an opportunity to come in contact with the iron and thus be absorbed to form the phosphite of iron, or ferrophosphorus.

To carry out the process of recovering the phosphorus, therefore, I prefer to withdraw the phosphorus bearing gases from the interior of the stack at a point or points in the lower region of the stack, as for instance, in the zone of tuyères, that is, the zone or vertical region extending generally from the bosh of the furnace to the slag line. In practice, however, it has been found that a somewhat more restricted zone extending a short distance upwardly from the level of the tuyères 100

is the most satisfactory from an operating standpoint, as there are less slag accretions to contend with and yet the gases in the region are sufficiently rich in phosphorus.

5 Any suitable means for withdrawing the gases from the furnace may be employed, the principal precaution to be observed being that of holding back the solid matter within the furnace while allowing the gas to pass 10 into the pipes or passages provided for the removal of the gases. The general procedure in withdrawing the gases is to tap the furnace wall at the point or points selected and to allow the gas to escape under the pressure 15 within the furnace. Practical furnace operators may readily devise suitable means for accomplishing this end.

The gases having been removed from the furnace are then treated, depending on the 20 use to be made of the phosphorus to be recovered. Such treatment would consist in general of a cooling the gas and condensing the phosphorus in several stages, as for instance, by passing the gas from one body of water to another, until the phosphorus content of the gases has been entirely condensed. A suitable operating equipment for this purpose would be a series of tanks filled with water, each having a discharge pipe near its 25 top which enters the succeeding container below the water level thereof, and so on. Thus each container will condense a portion of the phosphorus in the gases until it has all been removed.

15 Other means may also be employed for recovering the phosphorus, such as burning the uncondensed gas thereby converting the phosphorus into phosphorus pentoxide ( $P_2O_5$ ) and finally converting the  $P_2O_5$  into 20 phosphoric acid by treatment with water or water vapor and the recovery of the phosphoric acid from the gases by passing the same through an electric precipitator, as for instance, of the Cottrell type. However, any 25 suitable method of recovering the phosphorus or of treating the phosphorus thus recovered may be utilized without departing from the spirit of my invention.

It has also been observed that quantities 30 of phosphorus liberated within the stack of the furnace, find their way through the brickwork lining of the stack extending upwardly above the region of the tuyères to the down-comer, and also penetrates the 35 packing between the brickwork and the outer shell of the furnace. This phosphorus may also be removed from these portions of the stack aside from the regions immediately adjacent the tuyères, and hence I do not wish 40 to limit the invention to any specific region of removal, except perhaps at a level below the down-comer.

Having set forth a preferred method embodying my invention, I claim:

65 1. The process of recovering phosphorus

from phosphorus bearing material which comprises charging a blast furnace with phosphorus containing, and carbonaceous materials, and reducing and fluxing agents, and maintaining a high temperature and free carbonaceous material in the reducing zone of the furnace to reduce the phosphorus containing material to gaseous condition withdrawing the gases directly from said reducing zone, and recovering the phosphorus content from said gases.

2. The process of recovering phosphorus 70 from phosphorus bearing material which comprises charging a blast furnace with phosphorus containing materials, carbonaceous material and reducing and fluxing agents, maintaining a blast of heated air supply under pressure into the fusion zone of the furnace, to cause combustion of said carbonaceous material and produce and maintain a high temperature to enable the carbonaceous material to combine with the resulting phosphorus gaseous compounds to release their phosphorus content, withdrawing the resulting gases directly from said reducing 80 zone and recovering the phosphorus content 85 therefrom.

3. The process of recovering phosphorus 90 from phosphorus containing materials, which comprises charging a blast furnace with the phosphorus containing material and with carbonaceous materials, and reducing and fluxing agents, maintaining a phosphorus reducing temperature in the fusion zone of the furnace, to generate gaseous phosphorus containing compounds and enable the same to combine with the carbonaceous material to 95 release the phosphorus content thereof, then withdrawing the gases under pressure directly from the fusion zone of the furnace and recovering the phosphorus content therefrom.

4. The process of recovering phosphorus 100 from phosphorus containing materials, which comprises charging a blast furnace with the phosphorus containing material, and with carbonaceous materials, and reducing and fluxing agents, maintaining a phosphorus reducing temperature in the fusion zone of the furnace to generate gaseous phosphorus containing compounds and enable the same to combine with the carbonaceous material to release the phosphorus content thereof, then withdrawing the gases under pressure directly from the fusion zone of the furnace, 105 then cooling said gases and recovering therefrom the phosphorus content thereof.

5. The process of recovering phosphorus 115 from phosphorus containing materials which comprises charging a blast furnace with the phosphorus containing material, carbon, silica and iron containing material, subjecting the charged material to and maintaining a high reducing temperature in fusion zone 120 of the furnace to generate gaseous phos- 125

phorus containing compounds and enable the same to combine with the carbonaceous material to release the phosphorus content thereof, and withdrawing the gases directly from said fusion zone and recovering therefrom the phosphorus content thereof.

Signed at Nashville, Tenn., this 17th day of September, 1927.

JNO. W. WALTON.

10

15

20

25

30

35

40

45

50

55

60